

## UNITED STATES PATENT OFFICE.

ROBERT JAY SHOEMAKER, OF CHICAGO, ILLINOIS, ASSIGNOR TO S. & T. METAL COMPANY, OF CHICAGO, ILLINOIS, A CORPORATION OF ILLINOIS.

## ANTIFRICTION METAL.

No Drawing.

Application filed December 23, 1927. Serial No. 242,290.

My invention relates to anti-friction metals composed principally of lead and the object of the invention is to provide a hardened, toughened and stable alloy of lead 5 suitable for bearings, bushings or other elements where anti-friction properties are required or where, for other reasons, a hardened and toughened lead is required.

A further object is to provide a lead alloy 10 of this type which can be manufactured at low cost.

A further object is to provide a lead alloy which will not corrode when subject to moist atmosphere.

15 This application is a continuation in part of my copending application filed April 29, 1927, Serial No. 178,702.

The following examples will serve to illustrate the principles governing the compounding of the alloy of the present invention. Modifications will be suggested and these modifications and all embodiments of the invention within the scope of the appended claims are intended to be covered by 25 the patent.

*Example 1.*—This alloy is compounded of the following substances in the proportions by weight substantially as follows:

|           |                  |
|-----------|------------------|
| Calcium   | 0.1%             |
| Magnesium | 0.1%             |
| Tin       | 5.0%             |
| Aluminum  | 0.02% to 0.1%    |
| Lead      | to make up 100%. |

30 The alloy will have a hardness of approximately 19° Brinell. The magnesium appears to act as a hardener of the lead provided that tin is present. It does not seem to act as a hardener, at least to the same degree, if 35 tin is not present. If both substances are used, the magnesium lower limit may be 0.02%. The calcium may be varied from 0.1% to 1.0%. The tin may be used in quantities from 1.0% to 5.0%, but when in small 40 amounts the metal will lack hardness and when used in quantities above the upper limit specified, the alloy tends to become too brittle.

The aluminum plays no part as a harden-

ing agent, but tends to keep the calcium and magnesium from dropping out, when the alloy is melted and in compounding, and checks the tendency of the alloy to corrode when exposed to a moist atmosphere.

*Example 2.*—The alloy consists of the following substances in the proportions by weight substantially as follows:

|                       |               |
|-----------------------|---------------|
| Calcium               | 0.4%          |
| Magnesium             | 0.2%          |
| Aluminum              | 0.02% to 0.1% |
| Tin                   | 1.0%          |
| Lead to make up 100%. |               |

This alloy, because of its high calcium and magnesium content, and in spite of its low tin content, will have a hardness of from 21° to 25° Brinell. Both alloys as above specified are very tough. The ingredients of the alloy, preferred examples of which are given above, may vary within the ranges of 70 proportions as follows:

|                         |               |
|-------------------------|---------------|
| Calcium                 | 0.1% to 1.0%  |
| Magnesium               | 0.02% to 0.3% |
| Aluminum as stated, and |               |
| Tin                     | 1.0% to 5.0%  |

Larger quantities of aluminum can be used but the effect is detrimental, not beneficial. If more than 0.1% is employed, the excess will not go into solution and its presence tends to make the metal viscous when melted.

The alloy is compounded as follows:

The lead is first melted and heated to red 85 heat, approximately 1600° F. The melt is covered with a molten flux of calcium chloride. The tin and aluminum are introduced together as an aluminum tin alloy or consecutively as separate ingredients. The calcium is then stirred in followed by the magnesium. The temperature during these operations is maintained at substantially 1600° F. The metal is poured and the flux skimmed off. The calcium and magnesium 90 are put in in the form of sticks, lumps or bricks. Powder and turnings oxidize too 95 easily.

I claim:

1. Alloy consisting principally of lead and containing the following metals in quantities by weight substantially as follows: tin 1.0% to 5.0%; calcium 0.1% to 1.0%; magnesium 0.02% to 0.3%, and aluminum 0.02% to 0.1%.
2. Alloy consisting principally of lead and containing the following metals in quantities by weight substantially as follows: tin 10 1.0%; calcium 0.4%; magnesium 0.2%; and aluminum 0.02% to 0.1%.

ROBERT JAY SHOEMAKER.

**CERTIFICATE OF CORRECTION.**

Patent No. 1,703,212.

Granted February 26, 1929, to

ROBERT JAY SHOEMAKER.

It is hereby certified that error appears in the printed specification of the above numbered patent requiring correction as follows: Page 1, line 17, for "178,702" read "187,702"; and that the said Letters Patent should be read with this correction therein that the same may conform to the record of the case in the Patent Office.

Signed and sealed this 26th day of March, A. D. 1929.

(Seal)

M. J. Moore,  
Acting Commissioner of Patents.

I claim:

1. Alloy consisting principally of lead and containing the following metals in quantities by weight substantially as follows: tin 1.0% to 5.0%; calcium 0.1% to 1.0%; magnesium 0.02% to 0.3%, and aluminum 0.02% to 0.1%.
2. Alloy consisting principally of lead and containing the following metals in quantities by weight substantially as follows: tin 10 1.0%; calcium 0.4%; magnesium 0.2%; and aluminum 0.02% to 0.1%.

**ROBERT JAY SHOEMAKER.**

**CERTIFICATE OF CORRECTION.**

**Patent No. 1,703,212.**

**Granted February 26, 1929, to**

**ROBERT JAY SHOEMAKER.**

It is hereby certified that error appears in the printed specification of the above numbered patent requiring correction as follows: Page 1, line 17, for "178,702" read "187,702"; and that the said Letters Patent should be read with this correction therein that the same may conform to the record of the case in the Patent Office.

Signed and sealed this 26th day of March, A. D. 1929.

**(Seal)**

**M. J. Moore,  
Acting Commissioner of Patents.**